

## UNITED STATES PATENT OFFICE

ALBERT STAHN, OF HANOVER, GERMANY

## MAKING SAND CORES

No Drawing. Application filed April 5, 1928, Serial No. 267,799, and in Germany April 12, 1927.

My invention relates to cores for metal casting molds and more particularly to a binder for cores which consist principally or exclusively of pure quartz sand.

5 The cores of casting molds are either intended to remain in the mold in which they may have been formed, having been dried or burned while in the mold, or they are dried independently of the mold after the core box 10 has been removed.

My invention relates to cores of the latter kind which are dried independently of the mold. Heretofore such cores were made of earth containing clay and loam which 15 when mixed with water yield a plastic mass. Cores of any shape including complicated or undercut cores made from such earthy material will not collapse and will not undergo changes of form at normal temperature and in the kiln. However, these cores 20 involve certain drawbacks to wit:

1. The core is not sufficiently porous so that it is necessary to admix organic substances, such as dung, sawdust and the like 25 which impart porosity to the mass. It is, however, impossible to obtain in this manner uniform porosity so that the percentage of scrap is considerable.

2. The mass is not strong enough and the 30 core must therefore be reinforced by means of iron bars or wires which are difficult to remove from the finished casting.

3. In the kiln the core is burnt to the hardness of brick and must be removed from the 35 casting by means of hammer and chisel or by pneumatic tools.

In view of these and other drawbacks, cores made of earth are unsatisfactory. A core consisting principally or exclusively of 40 pure quartz sand, i. e. quartz grains of substantially uniform size, would be excellently suitable, but such cores could not be made heretofore for want of a suitable binder. Self-supporting cores must stand at normal 45 temperature without undergoing any deformation, even if they are very complicated, not even while being dried or burnt in the kiln. It has been attempted to provide a suitable binder but such attempts have failed, 50 as the binders were not able to fulfill the par-

ticular requirements of casting practice as follows:—The binder must be ready for use without requiring any preparation, in order to enable the core molder to make any number of satisfactory cores by mixing a predetermined quantity of quartz sand with a predetermined quantity of the binder. The binder must further remain unchanged for several months without its constituents separating.

55 The new binder according to this invention is a mixture of substances each of which has already been used separately or in combination with other substances, but none of these combinations aforesaid possesses the 60 properties required for a suitable quartz sand binder.

The new binder possesses the property of 65 imparting to the core such initial strength that insertions are only required in exceptional cases while on the other hand the core will immediately become disintegrated after casting and will flow from the casting in the condition of loose sand so that it is not necessary to remove it by special expedients.

70 My invention is based on the following considerations: In making a suitable core from quartz sand two binders are required, one of which should be soluble in water and the other in oil. The water-soluble binder must 75 impart to the core sufficient strength directly after it has been molded, by evaporation of the water and consequent incrustation of the surface of the core. The oil-soluble binder renders the dried core proof against the moisture of the mold and imparts to it the required high strength during drying notwithstanding a minimum percentage of binder used. Both binders should be reduced to a 80 minimum because any organic binder develops vapors or gases which may work damage 85 to the casting.

According to the present invention the two 90 binders are combined in such manner as to yield a stable mixture which is ready for use without preparation, the composition of 95 which does not change and the constituents of which do not separate. This is effected by combining the two constituents into a highly 100 viscous mixture which may have substan-

tially the consistency of dough or both substances are mixed initially in consistent condition. I thus obtain a binder, which may be stored for many months without undergoing any change as to its composition and it is therefore possible to withdraw small doses of the binder from a cask during several months without the portion which is used last, that is, the portion at the bottom of the cask, having other physical or chemical properties than the portions withdrawn at the beginning. Thus the core-maker need only admix per unit of weight of quartz sand the quantity of binder which has been determined once and for all, and he will always obtain a mass having the same plasticity and being invariable in shape at normal temperature and in the kiln. This is due to the fact that the binder will always and throughout its substance preserve those properties which were imparted to it initially. In this manner the principal drawback of existing binders of a similar character, to wit, the tendency of their constituents to separate sooner or later without this becoming outwardly apparent, is eliminated.

Two substances have been found to be particularly suitable for making the new core binder, the water-soluble substance being sulfite liquor, the oil-soluble binder being a pitch, more particularly stearin pitch. By mixing these two substances in highly concentrated condition a mixture is obtained which is almost plastic, is invariable for any length of time and possesses all properties required for making quartz sand cores, as set out above.

For instance a sulfite liquor of 35° Bé. which may still be concentrated if desired, is mixed with stearin pitch in the ratio of 30 to 70 parts of sulfite liquor and 70 to 30 parts of stearin pitch. Good results will be obtained by employing equal quantities of the two constituents.

The density of the mixture is higher than the density of each constituent. Quartz sand cores made with this binder are so strong initially that they may be placed on a conveyer and carried from the coremaker's stand to the kiln.

It is understood that I am not limited to any definite percentage of the two constituents, but the limits of percentages may be defined as follows:

1. The minimum percentage of highly consistent water-soluble binder such as is required for obtaining a core which will stand immediately upon molding and will not undergo changes of shape in the kiln, and the minimum percentage of highly consistent oil-soluble binder is such as required for obtaining high strength.

2. The minimum percentage of highly consistent water-soluble binder is such as required for obtaining a homogeneous mixture

of dough consistency with the highly consistent oil-soluble binder which must be permanent at any temperature.

These conditions determine the limits within which the percentages may be varied, and it will be understood from the wide range of proportions that the percentage cannot be fixed definitely being a function of the variable properties of the crude materials, of the purpose for which the binder is used, and of the ambient temperature which varies with the season.

Heretofore no binder was known which is ready for immediate use and may be transported to the works in casks, of which the coremaker has only to add to the quartz sand a predetermined quantity in order to obtain a self-supporting core and which does not undergo any changes during months.

Various changes may be made in the details disclosed in the foregoing specification without departing from the invention or sacrificing the advantages thereof.

I claim:

1. A highly viscous core binder consisting of sulfite liquor and an oil-soluble pitch.
2. A highly viscous core binder consisting of sulfite liquor and stearin pitch.
3. A metal casting core consisting of substantially pure quartz sand and a highly viscous mixture of sulfite liquor and stearin pitch.

In testimony whereof I affix my signature.

ALBERT STAHL.

100

105

110

115

120

125

130